

May 12, 1936.

R. J. WEAN

2,040,679

METHOD OF ANNEALING

Filed Oct. 15, 1935

2 Sheets-Sheet 1

*Fig. 1.*



*Fig. 2.*



INVENTOR

Raymond J. Wean  
by his attorneys  
Stebbins, Blenks & Parmelee

May 12, 1936.

R. J. WEAN

2,040,679

METHOD OF ANNEALING

Filed Oct. 15, 1935

2 Sheets-Sheet 2

Fig. 3.



Fig. 4.



INVENTOR

Raymond J. Wean

by his attorneys

Stebbins, Blenko & Parmelee

## UNITED STATES PATENT OFFICE

2,040,679

## METHOD OF ANNEALING

Raymond J. Wean, Warren, Ohio

Application October 15, 1935, Serial No. 45,083

2 Claims. (Cl. 266—5)

This invention relates to annealing and, in particular, to the annealing of material such as flat rolled steel products, i. e., sheets or strip in coils, although it has other applications.

5 The first step in the improvement of the art of annealing by the aid of the conventional annealing boxes which were charged bodily into annealing furnaces, was the development of a so-called bell or cover type furnace adapted to be lowered over a charge of material supported on a suitable base. The cover type furnace performs the same function as the annealing box cover, i. e., excludes the atmosphere to prevent oxidation of the material, and also furnishes the heat necessary for annealing. In order to prevent oxidation of the material upon removal of the cover, it was necessary to cool the furnace and charge to a temperature at which the oxidation would not proceed rapidly enough to be 10 objectionable, viz., about 1000° F. This meant that the furnace had to be kept over the charge for a long period after its heating function had been completed. This imposed serious limitations upon the capacity of a furnace of the bell type.

25 To overcome this limitation, it was proposed to place inner covers over the charge before lowering the furnace covers thereover. By this expedient, the furnace covers could be removed as soon as the charge had been raised to annealing temperature, and placed over a succeeding charge of material to be annealed, the inner cover being relied on to exclude the atmosphere during the cooling stage of the annealing cycle. Such inner covers are quite costly and have only a relatively limited 30 life, due to the extreme temperature conditions under which they operate, being subject directly to the furnace temperature during the heating cycle, and then to atmospheric oxidation while cooling.

35 40 I have invented a method and apparatus whereby the charge can be protected against atmospheric oxidation at all times without the necessity of subjecting the inner cover to the severe temperature conditions existing in the heating stage of the cycle. In accordance with my invention, I employ a furnace of the cover or bell type, but do not use the inner cover during the heating stage of the annealing cycle. The charge is brought up to annealing temperature with the 45 furnace cover thereover. The latter is then removed while the charge is at a temperature such that exposure to the atmosphere would result in objectionable oxidation of the material. A shielding cover similar to the inner covers now in use 50 is then placed over the charge to protect it from

the atmosphere. In the interim between the removal of the furnace cover and the lowering of the shielding cover, I protect the charge against oxidation by forming a curtain of non-oxidizing atmosphere on all sides thereof. Since the shielding cover is not subject to the furnace temperature during the heating stage of the annealing cycle, and is subject to the heat of the charge only during the cooling stage, the life of the shielding cover is much greater than that of the inner 10 covers heretofore used.

5 For a more complete understanding of the invention, reference is made to the accompanying drawings illustrating a present preferred embodiment of apparatus for practicing my invention. 15 In the drawings—

Figure 1 is a transverse sectional view of a bell type furnace having a charge therein ready to be annealed;

Figure 2 is a plan view of the furnace base 20 which supports the charge and receives the cover;

Figure 3 is a view similar to Figure 1, showing the charge on the base after the furnace cover has been removed and with the shielding cover in the course of being lowered over the charge; and 25

Figure 4 is a similar view showing the shielding cover in its final position.

Referring now in detail to the drawings, a bell type furnace 10 comprises a base 11 and a cover or bell 12. Both the base and cover have a refractory lining assembled within a structural frame. The furnace is similar in general to that shown in U. S. Patent No. 1,952,402. The joint between the base and cover is closed by a seal 13. A charge 14 of material to be annealed, in 35 this example, a stack of sheets, is supported on a bottom plate 15. A seal 16 surrounds the charge and is adapted to cooperate with a shielding cover to be described later.

40 The furnace 10 may be heated by any suitable means. Since the present invention is not concerned with the specific heating means employed, the latter has not been shown in detail, and may constitute the radiant tubes as shown in the patent aforementioned, or other heating means 45 such as electrical resistors or fuel burners.

45 A gas supply duct 17 is embedded in the lining of the base 11 and extends entirely around the bottom plate 15 outside the seal 16. A plurality 50 of nozzles 18 extend upwardly and inwardly from the ducts 17 at short intervals around the plate 15. Connections 19 extend laterally from the duct 17 to any convenient source of a non-oxidizing gas. This may be natural gas if such is 55

available, or any other suitable non-oxidizing gas.

Having described the apparatus of my invention, I will now explain the method practiced by the aid thereof. The cover 12 of the furnace is first removed from the base 11 to permit the charge 14 to be disposed thereon in the manner shown. The cover 12 is then replaced and the charge heated thereby to the annealing temperature. When the proper temperature has been reached, the cover 12 is removed. Substantially simultaneously with the removal of the cover 12 from the heated charge, non-oxidizing gas is supplied to the ducts 17 by operating suitable control valves. The nozzles 18 thus form curtains 20 of non-oxidizing gas on all sides of the charge. If the gas is combustible, it will be ignited on contact with the heated charge if sufficient air for combustion is present. This will be provided as the cover 12 is raised. So long as the supply of gas to the ducts 17 is continued, the curtains 20 protect the charge from atmospheric oxidation on all sides. The top sheet in the stack may suffer some oxidation, but this can be scrapped with but little loss or a special cover sheet can be placed on the top of the stack.

After the heating cover has been removed, a shielding cover 21 is placed over the charge as indicated in Figure 3. The lower edges of the cover 21 cooperate with the seal 16 and the atmosphere is thus effectively excluded from the interior of the cover. When the cover 21 has been lowered to the position shown in Figure 4, the gas supply for the ducts 17 may be cut off and the charge then permitted to cool in the normal way. The furnace cover, of course, is then lowered over a succeeding charge of material to be annealed and is thus operated with the highest efficiency, i. e., substantially continuously, in the performance of its function, viz., the heating of the material to be annealed to the proper annealing temperature.

The advantages of the invention will be apparent from the procedure that has been described. In the first place, the efficiency and capacity of the heating cover are not impaired

by the necessity for using it as a shield against atmospheric oxidation in addition to its heating function. Secondly, the shielding cover 21 is never subjected to the extreme temperature which exists on the inside of the furnace during the heating cycle and its life is therefore much greater than that of the inner covers as used heretofore. The maximum temperature to which the shielding cover is subjected is that of the fully heated charge, but this does not seriously affect the life of the cover since the charge starts to cool as soon as the heating cover is removed. The method and apparatus of my invention because of the increased life of the shielding covers as compared with that of the inner covers used previously, makes possible a material saving in cost over former practice.

Although I have illustrated and described herein but a preferred practice and embodiment of the invention, it will be apparent that changes therein may be made without departing from the spirit of the invention or the scope of the appended claims.

I claim:

1. In a method of annealing, the steps including disposing a charge of material to be annealed on a support, lowering a heating cover thereover to heat the material, removing the cover while the material is at a temperature such as to cause atmospheric oxidation thereof, discharging non-oxidizing gas adjacent the base of the charge to protect it against such oxidation, and then lowering a shielding cover over the charge to protect it from oxidation while cooling.

2. In a method of annealing, the steps including disposing a charge of material to be annealed on a support, lowering a heating cover thereover to heat the material, removing the cover while the material is at a temperature such as to cause atmospheric oxidation thereof, forming a curtain of non-oxidizing gas around the charge to protect it against such oxidation, and then lowering a shielding cover over the charge to protect it from oxidation while cooling.

RAYMOND J. WEAN. 45